

Patented Oct. 18, 1938

2,133,937

# UNITED STATES PATENT OFFICE

2,133,937

## COLOR PHOTOGRAPHY

Edmund B. Middleton and Andrew B. Jennings,  
New Brunswick, N. J., assignors to Du Pont  
Film Manufacturing Corporation, New York,  
N. Y., a corporation of Delaware

No Drawing. Application February 15, 1937,  
Serial No. 125,894

27 Claims. (Cl. 95—88)

This invention relates to color photography and more particularly to color-forming compounds which form dyes by coupling with the oxidation products of photographic developing agents.

A principal object of this invention is to provide a color-photographic element derived from color-forming compounds which, in combination with certain classes of developing agents, will form dyes in situ with photographic images. A further object is to produce such dyes by color-forming development. Another object is to produce partial color-records in which the individual records are of improved spectral quality for color photography.

It has been formerly taught to prepare colored photographs by developing exposed silver salt emulsion layers in certain developing agents whose oxidation products are water-insoluble dyes. Thus, a silver halide layer, bearing a latent image, can be developed in an alkaline indoxyl solution, whereupon a silver image is produced along with a blue dye image in situ with the silver. The silver image can be removed by Farmers Reducer revealing the dye image. In like manner, a photographic record can be developed in chlor-indoxyl to produce a green image and in thio-indoxyl for a red image.

It is also known, for the purpose of preparing color pictures, to develop exposed silver halide layers by agents whose oxidation products are not colored but which will chemically unite or couple with other organic agents, called "color-formers" to form intensely colored dyes. These "color-formers" are not photographic developers, are generally water-insoluble and produce dyes in situ with, and simultaneously with the deposition of the metallic silver image. The developers used for these proposed processes are of the diamino-aryl class, such as paraphenylenediamine or its substitution products, such as for example, di-methyl or di-ethyl-para-phenylene-diamine. Color-forming compounds already proposed include, for example, thymol, benzoyl acetone, phenacyl chloride and para-nitrobenzyl cyanide.

These prior processes, however, have failed to produce colored images having the correct spectral qualities for color photography. Moreover, these prior color-formers tend to have a harmful effect on the sensitivity of silver halide emulsions, so that, for these reasons, the color-formers already known have not provided a practical means for color photography.

The present invention has demonstrated that acylacetaminoarylmorpholines, in conjunction with aromatic amino developing agents, form satisfactory dye images. The acylacetamino-aryl-morpholines are aminoarylmorpholines wherein an amino hydrogen is replaced by the radicle of an acyl acetic acid, e. g., acetoacetic acid,

malonic acid, cyanacetic acid, furoylacetic acid, benzoylacetic acid and naphthoylacetic acid. The aminoarylmorpholines include the ortho-meta-and para-aminophenylmorpholines, amino-phenylthiomorpholines, aminonaphthylmorpholines, aminonaphthalithiomorpholines and their substitution products.

The acylacetaminoarylmorpholines may be made by condensing the ethyl or similar ester of the acylacetic acid with the aminomorpholine. 10

The following preferred examples are given as descriptive of the invention but not in limitation thereof:

Aceto-acet-p-aminophenylmorpholine  
HN.COCH<sub>2</sub>.COCH<sub>3</sub>



15

20

Aceto-acet-4-amino-2,5-diethoxy-phenyl-morpholine



25

30

35

Aceto-acet-p-amino-m-chlor-phenyl-morpholine



40

45

Aceto-aceto-p-amino-phenyl-thiomorpholine



50

55

The preferred color-forming compounds above 60

described may be used either in developers or as an addition to silver halide emulsions.

As preferred color-forming developers, the following produce excellent results:

5 *Formula 1*

|    |                                                        |       |     |
|----|--------------------------------------------------------|-------|-----|
|    | Diethyl-p-phenylenediamine hydrochloride               | gm    | 2   |
| 10 | Sodium sulfite, anhydrous                              | gm    | 5   |
|    | Sodium carbonate, anhydrous                            | gm    | 20  |
|    | Water to                                               | liter | 1   |
|    | To which is added aceto-acet-p-amino-phenyl morpholine | gm    | 1.0 |
| 15 | Ethyl alcohol                                          | cc    | 100 |

15 *Formula 2*

|    |                                                                     |       |     |
|----|---------------------------------------------------------------------|-------|-----|
|    | Diethyl-p-phenylenediamine hydrochloride                            | gm    | 2   |
| 20 | Sodium sulfite, anhydrous                                           | gm    | 5   |
|    | Sodium carbonate, anhydrous                                         | gm    | 20  |
|    | Water to                                                            | liter | 1   |
|    | To which is added aceto-acet-4-amino-2,5-diethoxy-phenyl-morpholine | gm    | 1.0 |
| 25 | Ethyl alcohol                                                       | cc    | 100 |

25 In place of the di-alkyl-substituted p-phenylenediamine, the mono-alkylated substitution procedure may be used or the un-substituted p-phenylenediamine may be used as well as the bases 30 and/or acid salts of these developing agents. In place of the ethyl alcohol, methyl alcohol or acetone may be used, and, if desired, the organic solvent for the color-forming compound may be dispensed with entirely.

35 If it is desired to add the color-forming compound directly to the emulsion, a preferred procedure is as follows: 10 grams of the color-former is dissolved in 200 mls. of ethyl alcohol to which is added about 50 grams of gelatin in 40 500 mls. of water and then thoroughly mixed. This color-forming solution is then added, with vigorous stirring, to 1 liter of silver-gelatino-emulsion. Emulsions containing these color-forming compounds may be coated as layers on 45 one or both sides of a photographic support either as individual or superposed emulsion layers.

While it is preferred to employ silver-gelatino-emulsions, other emulsions comprising other well 50 known sensitizers and binding agents may also be used. Examples of these are the well known silver collodion emulsion, albuminoid emulsion, or bichromated emulsion.

In the form of color-forming developers, the 55 above described compounds may also be used to re-develop bleached silver images. Thus, a silver image may be bleached in potassium ferrocyanide or a mixture of chromic and hydrobromic acids and re-exposed, whereupon the bleached 60 image can be re-developed to silver and a dye image by the color-forming developers above described. After development, the silver is removed by any of the well known reducers such as Farmers Reducer.

65 While the foregoing specification sets forth the preferred exemplifications of the present invention it is intended to include all variations and modifications within the spirit and scope of the appended claims.

70 We claim:

1. A color-forming photographic developer comprising an aromatic amino photographic developing agent and an acylacetaminoaryl morpholine.

75 2. A color-forming photographic developer

comprising an aromatic amino photographic developing agent and an acetoacetaminoaryl morpholine.

3. A color-forming photographic developer comprising an aromatic amino photographic developing agent and an acylacetaminophenylmorpholine. 5

4. A color-forming photographic developer comprising an aromatic amino photographic developing agent and an acetoacetaminophenylmorpholine. 10

5. A color-forming photographic developer comprising an aromatic amino photographic developing agent and acetoacet-p-aminophenylmorpholine. 15

6. A photographic developer comprising an N-alkyl-p-phenylenediamine and an acylacetaminoaryl morpholine.

7. A photographic developer comprising an N-alkyl-p-phenylenediamine and an acetoacet-20 aminoaryl morpholine.

8. A photographic developer comprising an N-alkyl-p-phenylenediamine and an acylacet-aminophenylmorpholine.

9. A photographic developer comprising an 25 N-alkyl-p-phenylenediamine and an acetoacet-aminophenylmorpholine.

10. A photographic developer comprising an N-alkyl-p-phenylenediamine and acetoacet-p-aminophenylmorpholine. 30

11. A color-forming photographic emulsion comprising a binding agent, a halogen salt of silver and an acylacetaminoaryl morpholine.

12. A color-forming photographic emulsion comprising a binding agent, a halogen salt of silver and an acetoacetaminoaryl morpholine. 35

13. A color-forming photographic emulsion comprising a binding agent, a halogen salt of silver and an acylacetaminophenylmorpholine.

14. A color-forming photographic emulsion 40 comprising a binding agent, a halogen salt of silver and an acetoacetaminophenylmorpholine.

15. A color-forming photographic emulsion comprising a binding agent, a halogen salt of silver and acetoacet-p-aminophenylmorpholine. 45

16. A color-forming photographic emulsion comprising a binding agent, a silver halide and an acetoacet-4-amino-2,5-diethoxyphenylmorpholine.

17. A color-forming photographic emulsion 50 comprising a binding agent, a silver halide and an acetoacet-p-amino-2-chlorophenylmorpholine.

18. A color-forming photographic layer comprising a sensitized gelatino-silver-halide emulsion and an acylacetaminoaryl morpholine. 55

19. A color-forming photographic layer comprising a sensitized gelatino-silver-halide emulsion and an acetoacetaminoaryl morpholine.

20. A color-forming photographic layer comprising a sensitized gelatino-silver-halide emulsion and an acylacetaminophenylmorpholine. 60

21. A color-forming photographic layer comprising a sensitized gelatino-silver-halide emulsion and an acetoacetaminophenylmorpholine. 65

22. A color-forming photographic layer comprising a sensitized gelatino-silver-halide emulsion and acetoacet-p-aminophenylmorpholine.

23. A color-forming photographic developer comprising an N-di-alkyl-p-phenylene diamine and an acylacetaminoaryl morpholine. 70

24. A color-forming photographic developer comprising an N-di-alkyl-p-phenylene diamine and an acetoacetaminoaryl morpholine. 75

25. A color-forming photographic developer comprising an N-di-alkyl-p-phenylene diamine and an acylacetaminophenylmorpholine.
26. A color-forming photographic developer comprising an N-di-alkyl-p-phenylene diamine and an acetoacetaminophenylmorpholine.
- 5 27. A color-forming photographic developer comprising an N-di-alkyl-p-phenylene diamine and acetoacet-p-aminophenylmorpholine.

EDMUND B. MIDDLETON,  
ANDREW B. JENNINGS.